

Feb. 6, 1940.

L. T. SIBLEY

2,189,409

LAMINATED SHEET MATERIAL

Filed Nov. 20, 1937

*Fig. 1*



*Fig. 2*



*Fig. 3*



*Fig. 4*



INVENTOR

Leon T. Sibley

BY

Alan N. Mann

ATTORNEY

## UNITED STATES PATENT OFFICE

2,189,409

## LAMINATED SHEET MATERIAL

Leon T. Sibley, Rutherford, N. J., assignor to  
 Alfol Insulation Company, Inc., a corporation  
 of Delaware

Application November 20, 1937, Serial No. 175,547

3 Claims. (Cl. 154—44)

My invention relates to laminated sheet materials and more particularly to a double reinforced, heat reflective water-resistant combined sheet material that will satisfactorily resist contraction and expansion caused by natural varying weather conditions, or by artificial varying conditions of humidity.

Numerous attempts have been made heretofore to produce combined paper sheet material that would be sufficiently waterproof to permit its use as a protective covering for structures or articles exposed directly or indirectly to varying humidity conditions. Also in connection with heat insulating materials various types of laminated paper and felt materials have been tried. As far as I am aware, all of these prior art laminated paper materials possess certain disadvantages that have seriously limited their commercial success. One of the main defects is that these materials are not waterproof and therefore will not withstand varying humidity conditions without becoming deformed or disintegrated.

One of the well known prior art paper materials, which is used for certain waterproofing and insulating purposes, consists of two heavy sheets of Kraft or similar heavy paper stuck together by means of a layer of asphalt or other adhesive with a matting of reinforcing fibers, commonly jute or sisal, imbedded in the layer of adhesive between the two sheets. This material has a dark dull surface which is conducive to heat absorption instead of heat reflection and its value as a heat insulating material is therefore negligible. It is to some extent water-resistant but does not prevent wetting of its fibrous portions when subjected to water or moisture vapor. These fibers as well as the paper itself on becoming wet tend to stretch and sag thereby causing the material as a whole to expand considerably in excess of its original size and area when normally dry; upon drying of the fibers as well as the paper itself the material will tend to shrink and contract to considerably less than its original size and area when normally dry. This expansion and contraction frequently causes a rupture of the paper. For this reason this material is limited in its effective use and particularly so where the use requires rigidly fastening the material so that it is not completely free to expand under wet conditions and contract under dry conditions.

As a specific example when the above described reinforced laminated paper is fastened by nails, tacks or the like over a shipping container as a protection to the container against the weather, as is commonly done, and is exposed to wet and dry weather or varying atmospheric humidity conditions, the paper will frequently contract to such an extent that it will pull away from the nails thereby breaking the fastening, frequently rupturing the paper itself, and rendering the

paper ineffective as a protective covering. Even if the paper does not entirely break loose from the container large openings will be formed around the nails which will permit water to enter the container.

An object of my invention is to provide a water-resistant, heat reflective, reinforced, combined sheet material that will resist contraction and expansion under varying moisture conditions.

In accordance with my invention I have made a reinforced sheet material that has a highly efficient heat reflective surface or surfaces, and is therefore an efficient heat insulator. It is highly water-resistant and accordingly will expand and contract only slightly with varying moisture conditions. Furthermore it is so constructed that this expansion and contraction will not adversely affect any of the combined sheets and will not break the bond between these sheets.

The sheet material of my invention, which is characterized by the above mentioned desirable features, comprises generally two assemblies of combined paper sheet and metal foil or other heat reflective material, laminated on opposite sides of a net of fibrous strands which are embedded in a thin layer of asphalt. In developing this finally commercially satisfactory product, which possesses unusual heat insulation moisture vapor and water-resistant properties, I made and tested several other types of laminated sheet materials all of which proved to be unsatisfactory. One of these materials consisted of two sheets of paper bonded together with adhesive and covered on both sides with sheets of metal foil. Contraction and expansion of the paper sheets under varying moisture conditions caused the metal foil covering to wrinkle and split in numerous places thereby losing its effectiveness as a waterproof covering. Another of the tested materials was like the one just described except that reinforcing fibrous strands were used between the two combined sheets in one direction. Contraction and expansion of the paper sheets in this material caused the metal foil covering to wrinkle and split along the fibrous strands which rendered the material unsatisfactory.

I finally discovered that by using a fibrous net as the reinforcing center member and by so positioning the paper metal foil assemblies on this net that a slight excess of paper and foil of each assembly sheet is provided around each of the net strands, the metal foil covering would not wrinkle or split and no other harmful effects would occur under varying moisture conditions. The apparent secret of success of this construction is that the excess material around each net strand under dry conditions will be used to compensate for the slight expansion that takes place in each of the small confined areas of the sheet under wet conditions. Each area, approximately one-half

inch square is bounded on all sides by the fibrous net strands. The excess material bridges each strand. Expansion or contraction of the sheet is basically limited to each small area because of the fibrous strands that bound and enclose each area. Therefore, movement of the material is confined to each small area which effectively prevents establishing a progressive stress throughout the sheet such as normally occurs in the prior art materials thereby causing rupture of the paper. The excess paper and foil bridged over each strand and the flexible and compressible nature of the strands compensate for slight movements of the material in each area, thereby preventing the paper and foil from rupturing due to those movements. Accordingly, there is insufficient stress set up between the paper, foil, and/or fibrous net strands over the entire area of the sheet during contraction or expansion to cause wrinkling or splitting of the foil, or rupture of the sheet.

Regarding the method of assembly of the product of my invention, I found that the metal foil or other heat reflective material could not be applied, with satisfactory results, to paper sheets previously combined and reinforced by the asphalt and fiber net. In other words this product cannot be obtained by simply covering laminated reinforced paper with metal foil or other heat reflective material, the main difficulty being that the foil cannot be applied uniformly and without wrinkling and splitting. The method that I finally determined upon as being commercially satisfactory comprises first combining the paper and heat reflective material by means of a suitable adhesive and pressing through rotating rolls and then combining these assemblies by means of adhesive with the center fiber net. The complete assembly is passed through rotating rolls and is compressed and dried. Passing through these last rolls effectively forms the paper and foil or other heat reflective material assemblies around the fiber net strands, thereby providing along each strand the excess of paper and heat reflective material required to compensate for contraction or expansion under varying moisture conditions.

The novel features of my invention are set forth with particularity in the appended claims. The invention itself however, both as to construction and method of assembly of the sheet material will be easily understood from the following description taken in conjunction with the accompanying drawing, in which:

55 Fig. 1 is a plan view, partly broken away, of one specific form of the material of my invention;

Fig. 2 is a sectional view taken along lines 2—2 of Fig. 1 and illustrates the excess of paper and foil around the fiber strands under normally dry conditions;

Fig. 3 is a sectional view similar to Fig. 2 but illustrating the material under wet expanded conditions; and

Fig. 4 is a sectional view similar to Fig. 2, but illustrating the material after having been wetted and thoroughly dried out again.

Referring now to the drawing, which it will be understood shows an illustrative but non-limiting example of my invention, the product consists of essentially two outer metallic sheets 10 and 11 combined with two inner paper sheets 12 and 13 to form two assemblies, the paper sheets being separated by a reinforcing net of fibers 14 which extend both horizontally and longitudi-

nally. The net 14 is held in place and the paper sheets 12 and 13 are held together by means of a layer of asphalt or other suitable adhesive shown at 15 applied on the side of each of the paper sheets 12 and 13 opposite the metallic sheets 10 and 11. The metallic sheets 10 and 11 are secured to the outer surfaces of the paper sheets 12 and 13 by means of any suitable type of adhesive indicated at 16.

The metallic sheets 10 and 11 may be made of any suitable flexible sheet metal such as for example aluminum foil, or any heat reflective material coating either metallic or non-metallic may be substituted for the metallic sheets. These sheets present a shiny exposed surface which is highly heat reflective thereby making the material of my invention particularly suitable for heat insulating purposes. Furthermore, these metallic sheets are substantially waterproof which renders the entire laminated sheet assembly highly resistant to water and the effects of varying moisture conditions. The thickness of these sheets or coatings may vary widely. One specific but non-limiting example is a foil of about 0.00035" in thickness. The metal foil sheets 10 and 11 show practically negligible contraction and expansion with varying weather or atmospheric humidity conditions, and therefore avoid the numerous difficulties encountered with the prior art types of laminated sheet materials having paper coverings.

The paper sheets 12 and 13, which according to my invention are covered with metal foil sheets or other heat reflective material may be made of any suitable relatively thin paper. I have found it advantageous to make these sheets relatively thin compared with the usual heavy paper and paper board heretofore used in order to reduce substantially the usual tendency of these thick sheets to contract and expand appreciably with varying moisture conditions. I have found that by making the sheets 12 and 13 of relatively thin paper, for example one specific but non-limiting thickness is 0.003", they will have appreciably less tendency to change in dimensions with varying weather conditions. These thin paper sheets could not be used in the prior art laminated paper materials because of their mechanical weakness and water permeability. In the material of my invention, however, they can be used since they are covered and protected by the waterproof metal foil or other heat reflective material sheets 10 and 11.

The fiber net consisting of crossed longitudinal and horizontal strands 14 may be composed of any suitable fibrous strands such as for example hemp or sisal. Likewise the arrangement of these fibrous strands may vary widely. All of the strands may be uniformly arranged or only part of them as indicated in Fig. 1.

The usual adhesive for laminating the paper sheets and for holding the reinforcing net in place is asphalt. In the assembly of my invention I have found asphalt to be entirely satisfactory for this purpose, but any other suitable adhesive having sufficient bonding power to hold the laminated sheets together may be used. An example of a suitable adhesive for sticking the outer metal sheets 10 and 11 to the inner thin paper sheets 12 and 13 is sodium silicate. Other suitable adhesives for example, converted starch adhesives, gutta percha cement, etc., may be used.

The important feature of providing an ex-

cess of paper and heat reflective material around each fiber strand 14 under normally dry conditions is shown in Fig. 2, and the use of this material under wet expanded conditions is shown in Fig. 3. Referring first to Fig. 2, it will be noted that the paper sheets 12 and 13 with their attached foil sheets 10 and 11 extend over and in contact and bridge the top and bottom surfaces of the strands 14 of the reinforcing net. This is illustrative of the excess amount, i. e. length and width, of sheet material when the product of my invention is used under normally dry conditions, conducive to negligible expansion or contraction of the entire sheet. It will be noticed that under this condition the combined paper and foil assembly is more or less in excess of a true flat area, around and over the strands 14.

Now, when the product is exposed to water, moisture vapor or other wet conditions normally conducive to expansion and sagging of the paper sheets the excess bridged material around the strands 14 is used up by its tendency to flatten out and elongate, and the sheet assemblies assume the lengthened condition illustrated in Fig. 3. There is now no appreciable excess of material formed around the strands 14. It will also be noted in this figure that the strands 14 have been compressed slightly from their normal round form shown in Fig. 2 to a more or less elliptical form. This also helps to prevent rupture of the sheet material upon expansion.

In Fig. 4 there is illustrated the material after being wet and dried. It will be noted that the contraction of the sheet results in humps of the foil and paper around the net strands even in excess to that present under normally dry conditions shown in Fig. 2.

While I have expressed above my understanding or theory of how the product of my invention reacts under varying moisture conditions to give satisfactory use, I wish it to be understood that my invention should not be limited to this or any other theory. Whatever the correct explanation is, the important fact is that the product does give satisfactory results under wet and dry weather conditions and thereby constitutes a substantial improvement over the materials tested and tried heretofore.

One of the commercial uses for which my product has proven particularly adaptable is in the insulation of railroad cars. In these cars and especially refrigerator cars the insulating material which lines the inner walls is subjected to varying degrees of moisture and unless the material is capable of withstanding these changes it will tear or disintegrate and lose its effectiveness as an insulator. The laminated sheet material of my invention is substantially waterproof and will therefore withstand subjection to these wet refrigeration conditions. Its light metallic or other heat reflective surface provides efficient heat reflection and therefore resists the transfer of heat through the railroad car walls. Furthermore, it is of sufficient stability and rigidity to permit its use without supporting frames or panels. It may be installed by simple attachment to cross members at top and bottom, thereby saving material and labor. It uses no felt or other type of mass insulation material and therefore avoids the defects of water and heat ab-

sorption and space requirements characteristic of mass insulation.

Another important commercial use of my product is in building insulation, particularly in air-conditioned residences and buildings. For this purpose the sheet material is placed directly behind the laths and plaster and will prevent the infiltration of moisture laden air into the wall or roof structure of the building, whereby insulation against heat and moisture is obtained.

From the foregoing description it will be understood that the material of my invention comprises principally a plurality of flexible heat reflective waterproof metallic sheets or non-metallic coating joined together in superimposed relationship through the intermediary of a plurality of relatively thin paper sheets adhesively fastened together and reinforced by a matting of fibrous strands.

As suggested hereinabove, it will be understood that my invention is not limited to the specific embodiments shown and described, but is subject to various modifications and changes as to size and type of materials and their method and arrangement of formation, including a laminated product of generally similar construction to the product shown except for use of the heat reflective sheet or coating on only one side of the material.

I claim:

1. A foil covered, reinforced, laminated sheet material which will permit limited relative movement under varying moisture and temperature conditions without splitting or otherwise adversely affecting the foil comprising two sheets of relatively thin paper, an intermediate net of reinforcing vegetable fiber strands having a thickness substantially greater than that of the paper sheets, said net being interposed between said paper sheets and bonded thereto by a layer of adhesive which also holds said sheets together, a relatively thin metallic foil covering the outer surface of at least one of said paper sheets, said paper sheets and foil covering being firmly pressed against said fiber net so that the crossing strands of the net form a network of crossing ridges in the paper and foil sheets, which correspond in number and distribution to the fibrous strands of the net and subdivide said sheets into a plurality of small areas bounded on all sides by said ridges, said ridges serving to confine within each respective small area the contraction and expansion of the material in said area which effectively prevents a progressive stress being established throughout the sheet, each of said ridges having an excess of paper and foil that bridges each of said fiber strands so that with varying moisture and temperature conditions the excess paper and foil may elongate across the fiber strands of each area and contract around the strands of each area without deleteriously affecting the foil and paper.

2. A foil covered, reinforced laminated sheet material as defined in claim 1, in which each of the paper sheets is covered with aluminum foil.

3. A foil covered, reinforced laminated sheet material as defined in claim 1 in which each of the paper sheets has a thickness not substantially greater than about 0.003 inch and the foil is substantially thinner than the paper sheets.

LEON T. SIBLEY.